

1

2,743,234

**STABILIZED SYNTHETIC LUBRICANT**

Alfred H. Matuszak, Westfield, and Ernest V. Wilson, Roselle, N. J., assignors to Esso Research and Engineering Company, a corporation of Delaware

No Drawing. Application June 25, 1954,  
Serial No. 439,478

11 Claims. (Cl. 252—46.7)

This invention relates to synthetic lubricating compositions. Particularly the invention relates to synthetic lubricating compositions which furnish satisfactory lubricating characteristics at both high and low temperatures. More particularly, the invention relates to synthetic lubricating oil compositions which have outstanding utility at both high and low temperatures and which comprise blends of a branched chain diester of a dibasic acid, a complex ester, phenothiazine and an amine.

In an effort to obtain superior lubricating oils having specific and unusual characteristics made necessary by the technical developments in the last few years, new synthetic lubricants have been developed by the art. One class of materials which has attracted unusual interest as synthetic lubricants are the esters, both the simple esters and the complex type. In general, these synthetic lubricating oils are characterized by lower volatility, higher viscosity indices, and lower pour points than mineral oils of a corresponding viscosity level. Lubricants possessing such properties are of special value in the lubricating of moving parts such as combustion turbines, particularly those of the "prop jet" and "turbo-jet" type for aircraft. Mineral oil lubricants containing added viscosity index improvers, pour point depressors, or other highly non-volatile additives are undesirable for use in such engines because of their tendency to leave a residue which accumulates and interferes with the operation of the turbine. Yet it has been found that these additive materials must be added to mineral oils to give them viscosity characteristics essential for operating at the extreme temperature differentials experienced. The synthetic lubricants of the ester type are especially adaptable for use under such conditions since these lubricants have a desirable combination of low volatility, low pour points, and high viscosity indices.

New design "turbo-jet" and "turbo prop" engines featuring high compression ratios and increased power output have forced temperatures upward and have increased the load on gears and bearings. Oil cooling has also become a problem since bearing temperatures in excess of 450° F. are not uncommon. These factors subject the lubricant to extremely severe conditions with regard to high temperature performance and load handling ability in addition to the ordinary low temperature requirements. Lubricants designed for these engines, therefore, must exhibit an outstanding combination of physical and chemical properties.

As the temperature increases the lubricant tends to thin out or decrease in viscosity. It is essential, however, that at the high temperature experienced the lubricant retain sufficient viscosity to furnish the lubricity necessary for decreasing friction. It has been found that in these new design engines, the viscosity of the oil at 210° F. and at 100° F. should be at least 3.0 and 11.0 centistokes respectively.

The load carrying ability of lubricants designed for these new uses must be adequate to properly lubricate the main anti-friction bearings at high speeds. This is

2

particularly true for the reduction gear assembly found in the turbo prop engines. Exhaustive tests have shown that the load carrying capacity for a lubricant for this use should be such as to result in a Shell 4-Ball seizure point of about 70 kilograms and a weld point of about 120 kilograms, both values given being minimum values. The explanation of the Shell 4-Ball test is set out in detail below.

In order to prevent excessive oil consumption the lubricant must possess a sufficiently low volatility. The ASTM flash point is used as a measure of volatility and it has been found that lubricants possessing flash points in excess of about 390° F. have been found to be satisfactory in this respect.

15 The viscosity of the oil at the minimum starting temperature of the engine must be sufficiently low as to prevent serious reduction in the oil flow rate. The maximum viscosity of the oil which can be pumped in adequate quantity has been found to be about 14,500 centistokes at —65° F.

It is generally recognized, therefore, that in order to furnish satisfactory lubrication of the new design turbo jet and turbo prop engines that a lubricant should have a viscosity at 210° F. of at least 3.0 centistokes, a viscosity at 100° F. of at least 11.0 centistokes, a viscosity at —65° F. of no more than 14,500 centistokes, and a load carrying capacity sufficient to obtain a Shell 4-Ball Extreme Pressure test seizure load of about 70 kilograms and a weld load of 120 kilograms.

20 It has been found, and forms the object of an application for Letters Patent, Serial Number 316,732, filed October 24, 1952, that blends of diesters and complex esters in conjunction with load carrying additives, exemplified by tricresyl phosphate, are especially adaptable for uses at high and low temperatures where extreme pressure resistance is desired. The instant invention represents an improvement of the blends covered in the above entitled application.

25 It has now been found that blends of diesters with complex esters as set out in detail in the copending application referred to above can be greatly improved especially in regard to lead corrosivity by incorporating therein a minor amount of practical grade phenothiazine as the oxidation inhibitor which also serves as an effective lead corrosion inhibitor.

30 It has been found, as data set out below will show, that pure phenothiazine is not nearly so adaptable as a lead corrosion inhibitor as is the practical grade phenothiazine. Hence it is desirable, from both the point of view of economics and increased effectiveness to use 35 the commercially available practical phenothiazine as both the oxidation and corrosion inhibitor for the blends to be more completely described below. The practical phenothiazine, which is dark green in color, is the product obtained by heating diphenylamine with sulfur and a trace of iodine catalyst. No purification treatment other than possible solvent stripping is involved. When the practical pheno is recrystallized from acetone-water mixture, pure phenothiazine, yellow in color, results.

40 When practical, or commercial grade, phenothiazine is blended with the compositions as an oxidation and corrosion inhibitor, it has been found that often a dark, objectionable, sludgy deposit is formed during storage. This deposit forms after several days storage or after 45 exposure to light, and is believed to be due to the impurities in the practical grade of phenothiazine. Although the exact composition of the impurities is not known, analysis of this sludge shows that the deposits are the end products of these impurities and are not found when pure phenothiazine is used as the oxidation inhibitor.

50 It is desirable, therefore, when employing phenothiazine as an oxidation inhibitor in synthetic lubricants

to use the practical grade material in order to take advantage of its increased corrosion inhibition. It is also desirable and equally important to overcome the problem of deposit formation since this sludgy material can lead to oil filter and oil line plugging, bearing deposits and eventual engine failure. The present invention has as its object the elimination of this objectionable sludge formation during the life of the oil.

It has been found that the inclusion in the synthetic lubricant formulation of minor amounts, in the order of from 0.001% to 5.0% by weight, based on the weight of the final formulation, of a primary, secondary or tertiary amine eliminates the problem of deposit formation. Although the exact nature of the phenomenon is unknown, it is believed that the amine compounds solubilize or neutralize the impurities, thereby preventing their deposition. The samples containing the amine materials remain clear and show no deposit formation after months of storage, even after exposure to light.

Thus, the instant invention has as its object new and useful lubricating compositions which comprise blends of mainly synthetic materials such as diesters of dibasic acids, complex esters prepared from alcohols, dibasic acids and glycols, phenothiazine of a commercial grade, and minor amounts of primary, secondary or tertiary aliphatic amines.

A more detailed description of the component parts of the compositions of invention is set out below.

#### THE BRANCHED CHAIN DIESTER

The dibasic acid which is fully esterified to form the diester portion of the lubricating oil blend may be selected from acids having the formula  $\text{HOOC}(\text{CH}_2)_x\text{COOH}$ ,  $x$  being 0 to 8. Preferred acids are sebacic, azelaic and adipic acid. These acids are well known in the art and need no further description.

The branched chain alcohol which is used to form the diester of the acid is selected from a group of alcohols which contains from 6 to 16 carbon atoms in branch chain configuration. It is essential that there be some degree of branching in the carbon chain of the alcohol, and, within limits, the higher the degree of branching the more satisfactory the lubricant. Alcohols such as ethylbutyl, ethylhexyl and other well known branch chain alcohols are operable.

One group of alcohols that have recently become commercially available and that answer the requirements for the esterifying alcohol are the so-called "Oxo" alcohols. These alcohols are preferred and are contemplated in the preferred embodiment of this invention.

The Oxo alcohols are prepared by the catalytic reaction of an olefin with carbon monoxide and hydrogen. The reaction, called "Oxo" synthesis, occurs at temperatures in the order of 300° F. to 400° F. at pressures in the range of about 1000 to 3000 p. s. i. In the presence of a suitable catalyst, ordinarily a heavy metal carbonyl, such as cobalt carbonyl, there is formed an aldehyde, which is subsequently hydrogenated to a primary alcohol. This process is described in U. S. Patent No. 2,327,066, issued to Roelen in 1943.

It has been found that particularly desirable alcohols for the esterification of the dibasic acid to prepare the diester component of the blend of this invention may be prepared by the application of the Oxo synthesis to polymers and copolymers of  $\text{C}_3$  and  $\text{C}_4$  monoolefins. These monoolefins are readily available in refinery streams and processes for their conversion to liquid copolymers and have been worked out by the art. One such process, known as UOP polymerization, consists of passing the olefin-containing stream in liquid phase in contact with an acid catalyst comprising phosphoric acid impregnated on kieselguhr. Other acidic catalysts, such as phosphoric acid or copper phosphate impregnated on silica gel, sulfuric acid, Friedel-Crafts catalysts, activated clays, silica-alumina, copper, pyrophosphate, etc., may be used.

Suitable conditions when employing phosphoric acid catalysts of the UOP type are temperatures of 300° F. to 500° F., pressures from 250 to 5,000 p. s. i., and feed stocks comprising refinery streams containing propylene and mixed butylenes. Suitable feed stocks, for example, may contain from 15 to 60 mol per cent propylenes, from 0.5 to 15 mol per cent butylenes, and from 0.1 to 10 mol per cent isobutylene, the remaining being saturated hydrocarbons. Other suitable feed stocks are the dimer and trimer of isobutylene.

Of the Oxo alcohols operable, those alcohols having from 6 to 16 carbon atoms are preferred. They are prepared from olefin polymers or copolymers having from 5 to 15 carbon atoms. In preparing these Oxo alcohols, the desired olefin fraction is segregated from the crude olefin polymer product by fractionation.

As was stated above, the Oxo alcohols are especially desirable esterifying alcohols because of their optimum degree of branching. For example, the following table shows the structure and percentage composition of a  $\text{C}_8$  Oxo alcohol prepared from a  $\text{C}_7$  olefin stream which had been fractionated from the products obtained by the phosphoric acid polymerization of refinery gas streams containing propylene and mixed n- and isobutylenes.

|    | Structure of $\text{C}_8$ "Oxo" alcohol                                                                                                                                                                                                                                             | Percent |
|----|-------------------------------------------------------------------------------------------------------------------------------------------------------------------------------------------------------------------------------------------------------------------------------------|---------|
| 30 | $\begin{array}{c} \text{C} \quad \text{C} \\   \quad   \\ \text{C}-\text{C}-\text{C}-\text{C}-\text{C}-\text{C}-\text{OH} \end{array}$                                                                                                                                              | 20.0    |
| 35 | $\begin{array}{c} \text{C} \quad \text{C} \\   \quad   \\ \text{C}-\text{C}-\text{O}-\text{C}-\text{C}-\text{C}-\text{OH} \end{array}$                                                                                                                                              | 25.0    |
| 40 | $\begin{array}{c} \text{C} \quad \text{C} \\   \quad   \\ \text{C}-\text{C}-\text{C}-\text{C}-\text{C}-\text{C}-\text{OH} \\ \quad \quad \quad \text{C} \\ \quad \quad \quad   \\ \text{C}-\text{C}-\text{C}-\text{C}-\text{C}-\text{C}-\text{OH} \end{array}$                      | 17.0    |
| 45 | $\begin{array}{c} \text{C} \\   \\ \text{C}-\text{C}-\text{O}-\text{C}-\text{C}-\text{C}-\text{C}-\text{OH} \\ \quad \quad \quad \text{C} \\ \quad \quad \quad   \\ \text{C}-\text{C}-\text{C}-\text{C}-\text{C}-\text{C}-\text{OH} \end{array}$                                    | 18.0    |
| 50 | $\begin{array}{c} \text{C} \\   \\ \text{C}-\text{O}-\text{C}-\text{C}-\text{C}-\text{C}-\text{OH} \\ \quad \quad \quad \text{C} \\ \quad \quad \quad   \\ \text{C}-\text{O}-\text{C}-\text{C}-\text{C}-\text{C}-\text{OH} \end{array}$<br>Alpha-alkyl-alkanols.....<br>Others..... | 2.3     |
|    |                                                                                                                                                                                                                                                                                     | 1.4     |
|    |                                                                                                                                                                                                                                                                                     | 4.3     |
|    |                                                                                                                                                                                                                                                                                     | 5.0     |
|    |                                                                                                                                                                                                                                                                                     | 100.0   |

It will be noted that Oxo alcohols derived from the olefins produced by  $\text{C}_3$ - $\text{C}_4$  polymerization are mostly methyl substituted.

Of the preferred Oxo alcohols operable as the acid esterifying agent, that is, those Oxo alcohols having from 6 to 16 carbon atoms, especially preferred are those Oxo alcohols having from 6 to 9 carbon atoms, that is, the  $\text{C}_6$  Oxo alcohol, the  $\text{C}_7$  Oxo alcohol, the  $\text{C}_8$  Oxo alcohol and the  $\text{C}_9$  Oxo alcohol.

#### THE COMPLEX ESTER

The second component of the synthetic lubricating compositions of this invention is generally known to the art as a "complex" ester. This material may be generally described as being the reaction product of two or more of the following compounds:

1. Monohydric alcohols
2. Monobasic acids
3. Dibasic acids
4. Glycols
5. Polyhydric alcohols
6. Polybasic acids

where at least one polyfunctional alcohol and at least one polyfunctional acid are employed.

These complex esters may be grouped under the following types:

**Type I.—Monobasic acid-glycol-dibasic acid-glycol-monobasic acid**

This complex ester may be considered to have the following structural formula:



wherein  $R_1$  and  $R_5$  are the alkyl radicals of the monobasic acids;  $R_2$  and  $R_4$  are the alkyl radicals of the glycols, and  $R_3$  is the alkyl radical of the dibasic acid.

The esters of this type may be prepared by admixing the calculated amounts of the various compounds and carrying out a straightforward esterification reaction. The reaction conditions are continued with an occasional sample of the product being tested for acidity until the minimum acidity is attained.

**Type II.—Alcohol-dibasic acid-glycol-dibasic acid-alcohol**

This ester, especially preferred among all the complex esters, has the following general formula:



wherein  $R_1$  and  $R_5$  are the combining radicals of the alcohol,  $R_2$  and  $R_4$  are the alkyl radicals of the dibasic acid, and  $R_3$  is the alkyl radical of the glycol.

These esters are prepared as those of Type I above, but preferably they are prepared by first forming the half-ester of the dibasic acid and the alcohol, and subsequently reacting two mols of such half-ester with one mol of the glycol.

**Type III.—Alcohol-dibasic acid-glycol-monobasic acid**

This ester may be represented by the following formula:



wherein  $R_1$  is the alkyl radical of the alcohol,  $R_2$  the alkyl radical of the dibasic acid,  $R_3$  the alkyl radical of the glycol, and  $R_4$  the alkyl radical of the monobasic acid. This ester may be prepared as described in Type I or it may be prepared by reacting a dibasic acid and a glycol under such conditions that one hydroxyl group of the glycol combines with one carboxyl group of the dibasic acid, in other words, so that a half-ester is formed. This half-ester is then reacted with a molar proportion each of an aliphatic alcohol and a monobasic acid.

**Type IV.—Monobasic acid - glycol - dibasic acid - glycol - monobasic acid**

These synthetic complex esters may be said to have the general formula:



wherein  $R_1$  and  $R_5$  are the alkyl radical of the monobasic acid,  $R_2$  and  $R_4$  are the alkyl radicals of the glycol, and  $R_3$  is the alkyl radical of the dibasic acid.

It will be noted that these esters are of the same formula as those appearing above under Type I, except that this type is prepared by reacting a monobasic acid with a glycol under such conditions that a half-ester is formed, and reacting two mols of such ester with one mol of a dibasic acid.

The alcohols used in forming the esters set out above include the following: methyl, ethyl, n-butyl, n-hexyl, n-octyl, 2-ethylhexyl, cetyl, oleyl, the ether alcohols formed by the reaction of ethylene oxide or propylene oxide with aliphatic alcohols, etc. One especially suitable group of alcohols are the Oxo alcohols described in detail above.

Among the monobasic acids which may be employed in the preparation of the complex esters the following may be listed as illustrative: acetic, propionic, butyric, valeric, capric, caprylic, pelargonic, lauric, palmitic, stearic, oleic, beta-methoxypropionic, beta-ethoxypropionic, beta-tert.-octoxypropionic, beta-ethylmercaptopropionic, beta-tert.-octylmercaptopropionic, beta-tert.-dodecylmercaptopropionic acid, and any of the various Oxo acids.

The glycols employed in preparing the complex esters referred to include ethylene glycol and any of the paraffinic homologues of the same containing up to about 18 carbon atoms. These may include, for example, ethylene glycol, propylene glycol, butylene glycol, pinacone, trimethylene glycol, tetramethylene glycol, pentamethylene glycol and the like. Since the glycols may also contain oxygen or sulfur atoms, compounds such as diethylene glycol, triethylene glycol and the polyethylene glycols of the formula:



wherein  $n$  is 1 to 26, may be used. Glycols containing sulfur atoms in thio-ether linkages include such compounds as thiadiglycol and 1,2 - bis(2 - hydroxyethylmercapto) ethane. There also may be used glycols containing both oxygen and sulfur in similar linkages; such a compound is bis-2-(2-hydroxyethoxy) ethyl sulfide.

The preferred embodiment contemplates an ester of Type II, for instance, one that is prepared by reacting two mols of a branched chain alcohol of from 6 to 16 carbon atoms with two mols of a half ester of a dibasic acid, such as succinic, glutaric, adipic, pimelic, suberic, azelaic, or sebacic acid, and one mol of a glycol such as polyethylene glycol. Specifically preferred is the reaction product according to the above procedure of 2-ethylhexanol, adipic or sebacic acid, and a polyethylene glycol of a molecular weight of about 200.

#### CORROSION INHIBITOR

One important characteristic essential in synthetic lubricants designed to operate at high and low temperatures is that they furnish satisfactory lubricity without undue corrosion of the bearing surfaces they lubricate. In order to enhance these characteristics various additive materials are blended into the finished formulation. Of these materials, one of the most satisfactory in regards to the inhibition of lead corrosion is phenothiazine of a commercial grade. As was pointed out above, chemically pure phenothiazine is somewhat lacking in its ability to prevent the corrosion of lead and it is difficult to meet existing specifications as to lead corrosivity levels with pure phenothiazine. It has been found, however, that impure, or commercial grade, phenothiazine, referred to as practical phenothiazine, is quite satisfactory in this respect. It has been found that inclusion in the finished diester-complex ester blend of from about 0.1 to about 2.0 weight percent, based on the weight of the finished composition, of practical or commercial phenothiazine results in a synthetic lubricant that gives very satisfactory lead corrosion results.

With the practical phenothiazine, however, the problem of deposit formation on storage develops. After storage of several days a black sludgy deposit develops which is believed to be due to the impurities present in the practical phenothiazine.

#### AMINE

The deposit formation problem occurring with the use of practical phenothiazine is solved according to the instant invention by inclusion in the formulation of from about 0.001 wt. percent to about 5.0 wt. percent, preferably about 0.1 to 0.5 wt. percent, of an amine of the formula



wherein R, R' and R'' are selected from the group consisting of hydrogen and alkyl groups containing from about 1 to about 24 carbon atoms. At least one alkyl group may contain a functional group selected from NH<sub>2</sub>, NHR and NR<sub>2</sub>, although these are not normally required. The preferred total number of carbon atoms in the amine will depend upon its volatility, solubility and effectiveness and will generally lie between 16 and 30 carbon atoms. Of the primary and secondary and tertiary amines operable in overcoming the deposit formation problem, the following are preferred.

Di-2-ethyl hexyl amine  
Bis(di-2-ethylhexyl amino) methane  
Armeens—C<sub>6</sub> to C<sub>24</sub> primary amine mixtures  
Trihexyl amine  
Octadecyl amine.

#### OTHER ADDITIVE MATERIALS

To enhance other characteristics of the synthetic lubricating compositions of this invention, other additive materials may be blended with the above to obtain a desired finished product. For example, load carrying properties may be enhanced by including from about 3 to about 10 wt. percent of tricresyl phosphate. Oxidation inhibitors, such as polynuclear phenols, alkylated phenols and the like in amounts varying from about 0.1 to about 2 wt. percent may be used.

Detergent inhibitors, such as petroleum sulfonates, or the metal salts such as the sodium, zinc, magnesium, barium, etc., salts of petroleum sulfonates in amounts of between about 0.1 and 8 wt. percent may be blended with the diester-complex ester blend serving as a base stock. From about 0.1 to about 5.0 wt. percent of rust inhibitors, such as polyhydroxy esters, e. g., sorbitan monooleate, and pentaerythritol monooleate, may be blended into the finished formulation. Lecithin may be used in amounts of between about 0.1 and about 2.0 wt. percent. Foam suppressants such as silicone fluids may be added in amounts up to about 0.1 wt. percent. Mineral oils in amounts of about 5.0 wt. percent to about 15.0 wt. percent or more may be added to aid in rust inhibition. Various other additive materials may be blended with the finished lubricant without departing from the spirit of the instant invention.

The invention will be more clearly explained by reference to the following illustrative examples.

#### EXAMPLE I

A synthetic lubricant blend was prepared by blending together 95 volume percent of the di-2-ethyl hexanol ester of sebacic acid with 5 volume percent of a complex ester prepared by reacting two mols of the half ester of 2-ethyl hexanol and sebacic acid with one mol of a polyethylene glycol of a molecular weight of about 200. To this blend was added 3.0 wt. percent of tricresyl phosphate as a load carrying agent. This blend is hereinafter referred to as blend A.

a. To blend A there was added 1.0 wt. percent of pure phenothiazine. One portion of this formulation was submitted to a lead corrosion test as follows:

Five hundred grams of the test oil was placed in a beaker equipped with a stainless steel stirrer and an inlet for bubbling air through the oil. On opposite sides of the stirrer there were affixed weighed strips of lead and copper. The oil was heated to a temperature of 325° F. with stirring and with air being blown through the sample. This temperature was maintained for one hour. At the conclusion of the test period the lead strip was removed, cleaned and the loss in weight calculated.

b. The second portion of the formulation was stored for 5 months and examined for sedimentation and color.

#### EXAMPLE II

a. To blend A there was added 1.0 wt. percent of practical, or commercially available, phenothiazine. One

portion of this formulation was submitted to the lead corrosion test detailed above and another portion was stored for 5 months and examined for deposit formation.

#### EXAMPLES III, IV AND V

To samples of blend A there was added 1.0 wt. percent of practical phenothiazine and 0.1 wt. percent of di-2-ethylhexyl amine (Example III), 1.0 wt. percent practical phenothiazine and 0.1 wt. percent of bis (di-2-ethylhexyl amino) methane, (Example IV) and 1.0 wt. percent practical phenothiazine and 0.1 wt. percent of a mixture of C<sub>12</sub>–C<sub>16</sub> primary amines (Example V). These formulations were divided into two portions; one of which was submitted to the lead corrosion test as set out above and the other of which was stored for 5 months and examined for sedimentation.

The results of the experiments performed on the samples as above are set out in the table below.

Table I

| Example No.                                                                                                   | Lead Corrosion (mg. wt. loss) | Months' Storage | Appearance after Storage in Light |
|---------------------------------------------------------------------------------------------------------------|-------------------------------|-----------------|-----------------------------------|
| 25 I. Blend A+1.0% Pure Phenothiazine.                                                                        | 30                            | 5               | Tan, No deposit.                  |
| II. Blend A+1.0% Practical Phenothiazine. Stored in dark.                                                     | 5                             | 5               | Tan, Heavy dark deposit.          |
| III. Blend A+1.0% Practical Phenothiazine+0.1% di-2-ethylhexyl amine.                                         | 5                             | 5               | Dark, Light deposits.             |
| IV. Blend A+1.0% Practical Phenothiazine+0.1% Bis (di-2-ethylhexyl amino) Methane.                            | 6                             | 5               | Light amber, No deposit.          |
| 30 V. Blend A+1.0% Practical Phenothiazine+0.1% C <sub>12</sub> –C <sub>16</sub> Primary Amine (Primene 81T). | 4                             | 5               | Amber, No deposits.               |
| 35                                                                                                            |                               |                 | Do.                               |

<sup>1</sup> Liquid reverts to original dark color on shaking but within a few hours' storage reprecipitates the sludge. The blend before storage, however, was dark but perfectly homogeneous. It showed signs of sludge formation after only several days' storage. This increased as storage time continued.

It will be seen that the material of Example III, IV and V, representing the inventive concept, exhibited excellent lead corrosion resistance in addition to showing no sedimentation after 5 months' storage. The pure phenothiazine, while giving no deposits, was lacking in satisfactory lead corrosion resistance.

Stoichiometric amounts of diphenyl amine (400 parts by weight) and sulfur (152 parts by weight) are heated in the presence of 0.3 part by weight of iodine as a catalyst to a temperature of about 190° to about 200° C. in a suitable reaction vessel. The heating is continued until the evolution of hydrogen sulfide ceases, usually for from 1 to 3 hours. The product is cooled and removed from the reaction vessel in the form of greenish crystals. This is the practical or impure grade of phenothiazine referred to hereinbefore.

In the purification of practical phenothiazine, the practical material is dissolved in acetone. After it is completely in solution, the addition of a small amount of water causes precipitation of the purer material. If the desired light yellow product is not obtained by one recrystallization, the operation may be repeated.

To summarize briefly, this invention relates to synthetic lubricating compositions which comprise blends of from about 20 to 95 volume percent of a diester of a dibasic acid containing from about 5 to about 16 carbon atoms in the ester group with about 80 to about 5 volume percent of a complex ester formed by reacting together at least three compounds of the group of C<sub>8</sub> to C<sub>18</sub> branched chain alcohols, dibasic acids, monobasic acids and glycols. To increase the resistance of the blends to lead corrosion there is added to them from about 0.1% to about 2% of a practical grade of phenothiazine and to eliminate deposit formation of the phenothiazine there is added from about 0.001 to about 5.0 wt. percent based

on the weight of the finished formulation, of an amine selected from the group consisting of primary and secondary and tertiary aliphatic amines. Other additive materials may also be incorporated into the finished formulation as will be recognized by those familiar with the art.

What is claimed is:

1. A synthetic lubricating oil composition which comprises a blend of from 20% to 95% by volume of a C<sub>6</sub> to C<sub>16</sub> branched chain alcohol diester of a dibasic acid with from 80% to 5% by volume of a complex ester formed by reacting together at least three compounds of the group of alcohols, monobasic acids, dibasic acids and glycols containing combined therein from 0.1 to 2.0 weight percent, based on the weight of the total composition, of impure phenothiazine which has been prepared by heating stoichiometric amounts of diphenylamine and sulfur to a temperature of about 190° to about 200° C. in the presence of iodine as a catalyst until evolution of hydrogen sulfide ceases, and from 0.001 to 5.0 wt. percent of an amine selected from the group consisting of primary, secondary and tertiary alkyl amines to prevent deposit formation from the commercial phenothiazine.

2. A synthetic lubricating oil composition according to claim 1 wherein said blend comprises 75 volume percent of the diester and 25 volume percent of the complex ester.

3. A composition according to claim 1 wherein said blend comprises 95 volume percent of said diester and 5 volume percent of said complex ester.

4. A synthetic lubricating composition according to claim 1 wherein said branched chain alcohols are the alcohols obtained by subjecting an olefin to the action of carbon monoxide and hydrogen at elevated temperatures and pressures in the presence of a cobalt catalyst.

5. A synthetic lubricating oil composition having a viscosity at 210° F. of at least 3.0 centistokes, a viscosity at 100° F. of at least 11.0 centistokes, and a viscosity at -65° F. of not more than 14,500 centistokes which comprises a blend of from 50 volume percent to 95 volume percent of a C<sub>6</sub> to C<sub>16</sub> branched chain alcohol ester of a dibasic acid selected from the group of adipic, azelaic and sebacic acid with from 50 volume percent to 5 volume percent of a complex ester formed by reacting two mols of a C<sub>6</sub> to C<sub>16</sub> branched chain alcohol half ester of a dibasic acid selected from the group of azelaic, adipic and sebacic acid with one mol of a polyethylene glycol, said blend containing combined therein from 2% to 10% by weight, based on the weight of the total composition, of tricresyl phosphate, from 0.1 to 2.0 wt. percent of impure grade phenothiazine which has been prepared by heating stoichiometric amounts of diphenylamine and sulfur to a temperature of about 190° to about 200° C. in the presence of iodine as a catalyst until evolution of hydrogen sulfide ceases, and from 0.001 to 5.0 wt. percent of an amine selected from the group of primary and secondary aliphatic amines to prevent deposit formation by the said phenothiazine.

6. A synthetic lubricant according to claim 5 wherein said blend comprises about 75 volume percent of said diester and about 25 volume percent of said complex ester.

7. A synthetic lubricant according to claim 5 wherein said blend comprises about 95 volume percent of said diester and about 5 volume percent of said complex ester.

8. A synthetic lubricant according to claim 5 wherein said branched chain alcohols are obtained by the action of carbon monoxide and hydrogen on an olefin at elevated temperatures and pressures in the presence of a cobalt catalyst.

9. A synthetic lubricant composition which comprises a blend of about 75 volume percent of di-2-ethylhexyl sebacate with about 25 volume percent of a complex ester prepared by reacting two mols of a C<sub>6</sub> to C<sub>16</sub> branched chain alcohol half ester of sebacic acid with one mol of a polyethylene glycol having a molecular weight of about 200, said blend containing combined therein from about 0.1 to about 2.0 weight percent, based on the weight of the total composition, of impure phenothiazine which has been prepared by heating stoichiometric amounts of diphenylamine and sulfur to a temperature of about 190° to about 200° C. in the presence of iodine as a catalyst until evolution of hydrogen sulfide ceases, and about 0.001 to about 5.0 weight percent of an amine selected from the group of primary, secondary and tertiary alkyl amines to prevent deposit formation from said phenothiazine.

10. A synthetic lubricating composition which comprises a blend of from about 20 volume percent to about 95 volume percent of a diester having the formula



wherein R and R' are branched chain alcohol residues containing from about 6 to about 16 carbon atoms and wherein x is a number of from 2 to 8, with about 80 volume percent to about 5 volume percent of a complex ester of the formula



wherein R and R' are branched chain alcohol residues containing from about 5 to about 16 carbon atoms, wherein x is a number of from 2 to 8, wherein y is a number of from 2 to 4, and wherein z is a number of from 1 to 6, said blend containing combined therein from about 0.1 to about 2.0 wt. percent of a commercial grade of phenothiazine which has been prepared by heating stoichiometric amounts of diphenylamine and sulfur to a temperature of about 190° to about 200° C. in the presence of iodine as a catalyst until evolution of hydrogen sulfide ceases and from about 0.001 to about 5.0 wt. percent of an aliphatic amine, selected from the group of primary, secondary and tertiary amines to prevent deposit formation due to the phenothiazine.

11. A synthetic lubricating composition which comprises a blend of a diester having the formula



wherein R and R' are branched chain alkyl groups containing from about 6 to 16 carbon atoms and wherein x is a number of from 2 to 8 with about 2.0% to 10.0% of tricresyl phosphate, about 0.1 to about 2.0% of a commercial grade of phenothiazine which has been prepared by heating stoichiometric amounts of diphenylamine and sulfur to a temperature of about 190° to about 200° C. in the presence of iodine as a catalyst until evolution of hydrogen sulfide ceases, and from about 0.001% to about 5.0% of an aliphatic amine.

#### References Cited in the file of this patent

#### UNITED STATES PATENTS

|    |           |                 |       |               |
|----|-----------|-----------------|-------|---------------|
| 60 | 2,190,648 | Cantrell        | ----- | Feb. 20, 1940 |
|    | 2,476,271 | Bartleson       | ----- | July 19, 1949 |
|    | 2,499,984 | Beavers et al.  | ----- | Mar. 7, 1950  |
|    | 2,639,266 | Dilworth et al. | ----- | May 19, 1953  |

#### OTHER REFERENCES

"Aliphatic Esters," Ind. and Eng. Chem., vol. 45, No. 8, pages 1766-1775, pages 1776 and 1767 pertinent.